

## UNITED STATES PATENT OFFICE

1,966,481

HOMOGENEOUS ANTIMONY-BISMUTH  
ALLOY

Pierre Berthelemy, Henry de Montby, and Jean-Marie Pouvreau, Paris, France, assignors to Société Anonyme française dite: Société des Brevets Berthelemy de Montby, Paris, France

No Drawing. Application February 17, 1933,  
Serial No. 657,262. In France October 29, 1929

2 Claims. (Cl. 75—1)

Messrs. Berthelemy and de Montby have shown that it is possible to incorporate homogeneously a metal such as cadmium into aluminium and aluminium alloys, by using magnesium as a vehicle for cadmium. This procedure brings about a perfectly homogeneous incorporation in well defined proportions, whereas if cadmium is introduced direct into the alloy, a heterogeneous incorporation results which makes it impossible 10 to obtain with certainty a determined proportion of cadmium.

Previous works seem to show that generally a metal is homogeneously distributed in other metals when such metal forms a solid solution 15 or a combination with these latter metals.

The researches of Messrs. Berthelemy, de Montby and Pouvreau have led them to discover that it is generally possible to incorporate homogeneously into aluminium and aluminium alloys 20 other metals which otherwise could only be incorporated heterogeneously, by using as a vehicle a metal capable of forming a solid solution or a combination with the metal to be incorporated, the latter having an affinity with aluminium. 25 Thus, lead, for instance, which while forming neither solid solutions nor compounds with aluminium, does form a solid solution with magnesium which in turn forms a solid solution with aluminium.

30 The object of this invention is to apply in industry this general method of incorporation into aluminium and aluminium alloys of an element which otherwise cannot be distributed homogeneously.

35 According to this invention, after preparing the alloy in the usual way and introducing its various ingredients, one adds a binary alloy consisting of the metal to be incorporated and that which is used as a vehicle.

40 As examples, the following binary alloys may be cited: antimony-bismuth, lead-magnesium etc.

The incorporation, however, can be carried out not only by using a binary alloy but also by 45 consecutive or simultaneous incorporation of the additional metal and the metal used as a vehicle. If the antimony and bismuth are not added to the aluminium in the form of a binary alloy, they should be added either simultaneously or in 50 such rapid succession as to form in effect a binary alloy, so that the antimony and the bismuth simultaneously act to cause them to be incorporated in the aluminium alloy, in the form of a solid solution.

55 It is to be clearly understood that the use

of the method of this invention does not exclude the addition of magnesium to the alloy, in cases where magnesium is no longer used as a vehicle for the metal to be incorporated.

The following are examples of alloy formulas 60 prepared according to the invention:

| Formula No. 1    |               |
|------------------|---------------|
| Silic. aluminium | Grammes 25 65 |
| Magnesium        | 9             |
| Antimony         | 10            |
| Bismuth          | 5             |
| Aluminium        | 951 70        |
|                  | 1000          |

| Formula No. 2    |            |
|------------------|------------|
| Silic. aluminium | Grammes 25 |
| Magnesium        | 9 75       |
| Bismuth          | 10         |
| Antimony         | 5          |
| Aluminium        | 951        |
|                  | 1000 80    |

| Formula No. 3    |            |
|------------------|------------|
| Silic. aluminium | Grammes 25 |
| Magnesium        | 9          |
| Lead             | 20 85      |
| Aluminium        | 946        |
|                  | 1000       |

If bismuth is added to aluminium a heterogeneous mixture is found however if the bismuth is simultaneously added with antimony to the aluminium, as in the form of a binary alloy, the joint action of the antimony and of the bismuth causes them to be distributed throughout the aluminium in the form of a solid solution, so that the antimony and the bismuth are 95 homogeneously distributed throughout the alloy.

Experiments have shown that bismuth is not miscible in aluminium save in very small proportions, as for example about 0.3%. By utilizing the antimony, a large proportion of bismuth can be homogeneously distributed in the final alloy. By reason of this uniform distribution, the applicant prevents the formation of electro-chemical couples, and this is highly desirable because such couples produce corrosion.

Since the bismuth is distributed in the alloy in a proportion which is much greater than the normal limit of about 0.3% due to the action of the antimony, the bismuth is retained in the 110

final alloy in the free state. The bismuth retains, therefore, its essential characteristics, so that the bismuth prevents the formation of electro-chemical couples.

5 The simultaneous incorporation of the bismuth and of the antimony therefore permits the bismuth to exercise what may be considered as being a physical action upon the final alloy.

This is contrary to the proposals made by previous inventors, in which it was suggested to add a small amount of antimony to the aluminium, in order to protect the aluminium against the action of salt water.

Prior inventors sought to add the antimony to aluminium in order to produce a surface formation of antimony oxychloride on the piece of aluminium.

Applicants restrain or prevent the corrosion of aluminium alloy by means which are essentially physical, in contradistinction to the chemical means previously utilized.

This application is a continuation in part of our application Ser. No. 488,987, filed in the U. S. Patent Office on October 15, 1930.

25 What we claim is:

1. A method of forming an aluminium alloy containing a major proportion of aluminium and also containing antimony and bismuth, which consists in adding an alloy of antimony and bismuth to the aluminium, so that the alloy takes up bismuth in excess of 0.3%, in the form of solid solution. 80

2. A method of incorporating antimony and bismuth in an alloy, the major part of which consists of aluminium, so that the antimony and the bismuth form solid solutions in the aluminium, which consists in adding the antimony and the bismuth to the aluminium substantially simultaneously, so that the antimony and the bismuth jointly act upon each other to form solid solutions of said antimony and bismuth in the aluminium, the bismuth being added in excess of 0.3%, and the percentage of antimony being sufficient to cause said excess to form said solid solution. 85 90 95

PIERRE BERTHELEMY.  
HENRY DE MONTBY.  
JEAN-MARIE POUVREAU.

100

30

105

35

110

40

115

45

120

50

125

55

130

60

135

65

140

75

150